

Oct. 9, 1951

E. R. ZADEMACH ET AL

2,570,299

PORCELAIN ENAMELING PROCESS

Filed Feb. 14, 1947



## UNITED STATES PATENT OFFICE

2,570,299

## PORCELAIN ENAMELING PROCESS

Erich R. Zademach and William W. Clarke, Hillside, N. J., assignors to Metalwash Machinery Company, Irvington, N. J., a copartnership

Application February 14, 1947, Serial No. 728,414

4 Claims. (Cl. 117—70)

1

The present invention relates to a method and apparatus for cleaning, pickling and nickel plating metal parts in preparation for the porcelain enameling thereof.

It has been the practice after metal parts have been cleaned and pickled, to immerse them in a bath of nickel sulphate solution to form thereon a coating of nickel to which the enamel is subsequently bonded. Hitherto, it was the common belief of the art that a good effective nickel coating to which enamel would strongly adhere could not be deposited on a metal object by any process except an immersion process.

One object of the present invention is to provide a new and improved process and apparatus for depositing a nickel coating on metal parts in preparation for the porcelain enameling thereof.

Another object is to provide a continuous process and apparatus by which metal parts may be effectively and quickly cleaned, pickled and nickel coated in preparation for porcelain enameling.

In accordance with certain features of the present invention, a nickel salt solution, such as that of nickel sulphate, is sprayed on the metal parts after they have been cleaned and pickled. It is found by actual impact tests, that the coating of nickel deposited on the metal parts by this spray process is such as to cause the porcelain enamel subsequently applied to said parts to adhere more strongly thereto, than in the case of a nickel coating applied by the immersion process.

As a further feature, the spraying of the nickel sulphate solution or other nickel depositing salt solution on the metal parts is combined with the spraying of the cleaning, pickling and rinsing liquids in successive stages in a continuous process and apparatus, thereby attaining maximum production capacity. Furthermore, with a continuous process and apparatus as described, the apparatus can be set to operate uniformly on all metal parts, without being affected by the operator's discretion, as in the case of a discontinuous immersion process or apparatus. All metal parts, therefore, will receive uniform treatment, and will be uniform in character when subjected to the porcelain enameling process. Furthermore, this process and apparatus not only results in superior cleaning, but since the air in the spaces between the operations in the apparatus is in liquid or vapor saturated condition, the work cannot dry out between the various treatments or stages, nor is it contaminated by being drawn up through the slime on the surfaces of the immersion tanks.

2

Various other objects, features and advantages of the invention will be apparent from the following particular description, and from an inspection of the accompanying drawings, in which:

Fig. 1 is a top plan view somewhat diagrammatic of the improved apparatus which embodies the present invention, and which can be employed to carry out the process of the present invention; and

Fig. 2 is a diagrammatic transverse section of the apparatus taken on line 2—2 of Fig. 1.

Referring to the drawings, there is provided a long treating chamber or tunnel 10, shown in the form of a J, to suit the available floor space, and having an opening or slot 11 in the roof 12 thereof extending along the length of said chamber. Extending along the top of the tunnel 10 over the slot 11 are the runs of an endless horizontal rail conveyor 13. Supported from this conveyor 13 and rolled along the rail thereof are hangers 15 from which the metal parts 16 to be treated are suspended. These metal parts 16, which are usually of iron, are shown in the form of flat plates, but it must be understood that as far as certain aspects of the invention are concerned, these may be of any suitable shape.

The tunnel or chamber 10 is divided into different compartments by partitions 18 having openings 20 through which the metal parts are continuously advanced edgewise. Suitable ventilators 19 are provided for the tunnel in the form of openings in the roof, especially between the spraying regions of the compartments.

The metal parts 16 are introduced into the tunnel 10 from the entrance end 21 thereof, and are advanced continuously therealong until they are discharged from the exit ends 22 thereof. As the metal parts are continuously advanced through the tunnel 10, they are subjected to different cleaning, pickling nickel plating and drying stages in sequence, as will be described.

Near the entrance end of the tunnel 10 is a compartment A, in which each metal part 16 is sprayed with a hot emulsion wash from two sets of spray units 23, located on opposite sides of the path of travel of said metal part. Each of these spray units 23 consists of a plurality of vertical headers having spray nozzles in the inner sides thereof, spaced therealong to project the spray jets 24 against the advancing metal object 16. The circulating system for the spray units 23 in the compartment A comprises a sump tank 25 into which the sprayed solution is drained,

and from which the spray solution is recirculated to the spray nozzles by a pump 26.

The hot emulsion spray wash in the compartment A removes the surface dirt and grease from the metal part 16, and comprises a suitable cleansing liquid, as for example, a mixture of kerosene and water containing cresylic acid or other appropriate emulsifying agent.

The metal work object 16 then advances into compartment B where said object is subjected to a fresh water spray rinse from spray units 27 on opposite sides thereof similar to those in compartment A, in order to wash off the dirt, grease and emulsifying liquid from the previous operation in compartment A. The fresh water is delivered to these spray units 27 by a feed line 28, and the spent water is drained to sewer by a discharge line 29.

The operation in compartment B may leave an oil film on the metal object. To remove this oil film, the metal object 16 is subjected to a hot alkali spray wash in compartment C from spray units 30 located on opposite sides of the course of said metal part, as in compartment A, and fed by a recirculating system comprising a sump tank 31 and a circulating pump 32 connected on its suction side to said tank, and on its discharge side to said spray units.

The metal object 16 then moves into the compartments D, where it is subjected to a three-stage water rinse to remove the residual alkali therefrom. In this compartment D, there are three groups of spray units 34, 35 and 36, each comprising a pair of or two sets of vertical headers on opposite sides of the path of travel of the metal object, and each carrying a series of spray nozzles. The first group of spray units 34 supplies recirculated rinse by means of a pump 40 from a recirculating sump tank 38 underneath the spray units 35 and 36, so that most of the residual alkali wash is removed from the metal object 16. The spent rinse water from the spray units 34 is drained to the sewer through a discharge line 37. The second group of spray units 35 supplies recirculated rinse water from the sump recirculating tank 38 by means of the pump 40, and the drain from said spray units is returned to said tank.

Clean fresh water from a supply line 41 is delivered to the third group of spray units 36 for a final rinse of the metal object 16, and is drained into the sump tank 38. This clear water rinse is controlled, so that it makes up the amount of water diverted and drained to sewer by the first group of spray units 34.

After rinsing in the compartment D, the metal object 16 moves into the compartment E, where it is subjected to the action of a hot pickling liquid, which is desirably 10 to 15% sulphuric acid solution. This sulphuric acid solution in the compartment E is sprayed on to the advancing metal object 16 by two sets of spray units 43, which are located on opposite sides of the path of travel of said object, and which are similar in construction to the other spray units described. The hot sulphuric acid solution is recirculated through the spray units 43 by a sump tank 44 and a pump 45.

The metal object then advances into the compartments F, which are similar to the compartments D, and in which the metal part is subjected to a three-stage water rinse as in said latter compartments.

The metal object after being thoroughly washed in the compartment F, travels into com-

partment G. In this compartment, the metal object 16 is subjected to a spray of a solution of a nickel salt of a character which has an anion capable of reacting with the ferrous metal of the object 16, to deposit a coating of pure nickel on to said object. The liquid usually employed for that purpose is nickel sulphate solution. This nickel sulphate solution is sprayed in the form of a mist on to the metal object 16 as it travels through the compartment G. The pressure of the solution in the spray headers may be between eight and ten pounds per square inch.

For the purpose of spraying the nickel sulphate solution on to the metal object 16, there are provided two sets of spray units 50 disposed on opposite sides of the course of travel of said object. Each of the spray units 50 comprises a series of substantially vertical headers 51 spaced along the compartment G, and interconnected by a feed line 52 on the discharge side of a recirculating pump 53, the suction side thereof being connected to a sump tank 54 at the bottom of the compartment, and in position to receive the drain from the spray units 50.

The nickel sulphate solution may be of any suitable strength, and may, for example, have a concentration of about two ounces of the hydrated sulphate  $\text{NiSO}_4 \cdot 6\text{H}_2\text{O}$  to one gallon of water or the equivalent of .448 ounce of nickel per gallon. The temperature of the nickel sulphate solution is approximately 175° F., and its pH is from 3 to 3.5. The metal object 16 may travel at a rate of five to ten feet per minute through the compartment G, and the time required to traverse said compartment may take from three to five minutes, during which time the metal object 16 is subjected to the spray of hot nickel sulphate solution. As a result of this operation, a coating of pure nickel is deposited on the surface of the metal object 16. This nickel coating will be of uniform thickness throughout the area of the metal object 16, and its characteristics will be predetermined according to the shape and size of the metal object, speed of travel thereof through the compartment G, the concentration and temperature of the hot nickel sulphate solution, and other factors, all of which may be easily controlled. It is found, for example, that for a nickel sulphate spraying period of three minutes, there will, under certain conditions, be deposited a nickel layer at the rate of .05 grams per square foot, and for a nickel sulphating period of five minutes, the nickel deposit will be at the rate of about .08 grams per square foot.

The metal object 16 after having the coating of nickel formed thereon by the spraying process described, passes through compartments H, where it is subjected to a three-stage water rinse spray, as in compartments D and F.

From the compartment H, the metal object 16 travels into compartment I, where it is subjected to a neutralizing spray to remove any residual acid thereon. The spraying in the compartment I is effected through two sets of spray units 56 disposed on opposite sides of the course of travel of the metal object 16, as in the other compartments, and the neutralizing solution is circulated through said spray units by means of a sump tank 57 and a pump 58. The neutralizing spray solution may consist of a combination of sodium carbonate and borax. The metal object 16 then travels into the final compartment J, where it is subjected to a hot blast from a series of hot air blast units on opposite sides of the metal object. The air for the pur-

pose is delivered by a fan 60 and is heated by a heater 61. The metal object 16 treated as described can, after leaving the tunnel 10, be dipped or sprayed with enamel and baked in the usual manner.

As an example, a time schedule of operations and the temperatures of the fluids employed in the different stages of operations, is indicated below for a specific installation. It must be understood that this schedule may be changed according to different operating conditions desired:

*Time and temperature schedule*

|                                  | Tempera-ture | Time                       |
|----------------------------------|--------------|----------------------------|
| (A) Emulsion wash.....           | ° F.<br>180  | Minutes<br>1 $\frac{1}{4}$ |
| (B) Water rinse.....             | Cold         | 1 $\frac{1}{2}$            |
| (C) Alkali wash.....             | 180          | 1 $\frac{1}{4}$            |
| (D) Water rinse.....             | Cold         | 1                          |
| (E) Sulphuric acid pickling..... | 160          | 2 $\frac{1}{2}$            |
| (F) Water rinse.....             | Cold         | 1                          |
| (G) Nickel sulphate spray.....   | 175          | 3                          |
| (H) Water rinse.....             | Cold         | 1                          |
| (I) Neutralizing.....            | 180          | 1 $\frac{1}{4}$            |
| (J) Air blast drying.....        | 220          | 5                          |

It should be noted from the above schedule of operations, that the periods of the various cycles are very much shorter than is the case with the usual type of immersion cleaning, pickling and nickel sulphating. Nevertheless, the cleaning results obtained are much superior to those obtained in the usual immersion processes. Furthermore, it has been shown by actual tests, that the enamel will adhere more strongly to the nickel coating deposited by the spray process than by the usual immersion process.

While the invention has been described with particular reference to a specific embodiment, it is to be understood that it is not to be limited thereto, but is to be construed broadly and restricted solely by the scope of the appended claims.

What is claimed is:

1. In a process for porcelain enameling a ferrous object in which a layer of nickel is first deposited thereon and the porcelain enameling subsequently formed on said nickel layer, the improvement which comprises conveying a substantially vertically disposed ferrous object through a directed mist of an aqueous solution of a nickel salt having an anion capable of unit-

ing with the metal in said object, said object being subjected to said mist for a period of at least three minutes, said aqueous solution being at a temperature of approximately 175° F., and draining the excess solution from said object by gravity flow.

2. In a process for porcelain enameling a ferrous object in which a layer of nickel is first deposited thereon and the porcelain enameling subsequently formed on said nickel layer, the improvement which comprises conveying a substantially vertically disposed ferrous object through a directed mist of an aqueous solution of a nickel salt having an anion capable of uniting with the metal in said object, said object being subjected to said mist for a period of at least three minutes, and draining the excess solution from said object by gravity flow.

3. In a process for porcelain enameling a ferrous object in which a layer of nickel is first deposited thereon and the porcelain enameling subsequently formed on said nickel layer, the improvement which comprises conveying a substantially vertically disposed ferrous object through a directed mist of an aqueous solution of a nickel salt having an anion capable of uniting with the metal in said object, and draining the excess solution from said object by gravity flow.

4. In a process for porcelain enameling a ferrous object in which a layer of nickel is first deposited thereon and the porcelain enameling subsequently formed on said nickel layer, the improvement which comprises conveying a ferrous object through a directed mist of an aqueous solution of a nickel salt having an anion capable of uniting with the metal in said object, and draining the excess solution from said object by gravity flow.

ERICH R. ZADEMACH.  
WILLIAM W. CLARKE.

REFERENCES CITED

The following references are of record in the file of this patent:

UNITED STATES PATENTS

| Number    | Name      | Date          |
|-----------|-----------|---------------|
| 2,064,173 | McGohan   | Dec. 15, 1936 |
| 2,265,467 | Alexander | Dec. 9, 1941  |
| 2,279,686 | Kerlin    | Apr. 14, 1942 |